

## UNITED STATES PATENT OFFICE.

GEORG GUDE GEDDA, OF SURAHAMMER, SWEDEN.

## MODE OF PRODUCING WROUGHT IRON WITH INCREASED TENSILE PROPERTIES.

No Drawing. Application filed December 9, 1925, Serial No. 74,408, and in Sweden July 17, 1925.

Wrought iron processes heretofore practiced, such for example as the triple melting-down process, the Walloon or half-Walloon process, the Lancashire, the covered refinery 5 and the puddling processes, have to a large extent been superseded by the ingot steel production, due partly to the fact that this has proven to be cheaper, and partly because it results in a product having its composition 10 so altered as to increase the tensile properties thereof.

To substitute the ingot iron for the wrought iron has, however, been impossible for certain purposes. This is the case, when 15 the welding capacity and the fibrous structure, qualities which are characteristic of the wrought iron, are of a decisive importance. The production of a wrought iron with its usual characteristic qualities, but 20 with an improved tensile strength, has long been sought. For this purpose an incomplete fining away of coal or manganese has been proposed but by this process the welding capacity is disadvantageously affected 25 and the process is very unreliable, also. It has also been proposed to use a pig-iron with a specially high percentage of phosphorous; in this case the whole phosphoric percentage is met with in the wrought iron, which 30 causes an improved tensile strength of the product, but also a greater brittleness and a greater unreliability. Experiments have been made with cold rolling, but because of its unreliability this mode is not practical, 35 at least when important construction materials are concerned. In these and other cases it has been possible to increase the elastic limit and to increase the maximum tensile strength, but the contraction and the impact 40 capacities have, on the other hand, always been decreased.

The problem of increasing the maximum tensile strength of the wrought iron, and also increasing its elastic limit, without a simultaneous and considerable reduction of its 45 welding capacity, as well as the impact and contraction capacities of the material, is solved by the present invention.

I have discovered that this may be attained by an alloying of the wrought iron with nickel. It may be accomplished in va-

rious ways. For example, as fining material, I may use a pig-iron, that previously has been alloyed with nickel, for instance by such means, that the nickel as pure metal 55 or as an alloy has been put in the charge used in the pig-iron production. The nickel may also be put in by such means, that the nickel, or a nickeliferous material, is placed in the finery or, it is possible by the use of 60 nickeliferous iron in such a way to increase the quantity of nickel. Nickel being a metal with considerably less affinity for oxygen than the iron, practically the whole quantity of nickel used will form a part of the 65 refined iron. In the slag there will only be traces of nickel.

A Lancashire bloom produced by the invention and containing 0,03% C, 0,01% Si, 0,07% Mn, 0,006% S, 0,021% P and 3,57% 70 Ni has, by analysis, proved to have a maximum tensile strength of 38,5 kg./mm.<sup>2</sup>, an elastic limit of 30-31 kg./mm.<sup>2</sup>, a contraction of about 75% and an impact test as per Charpy of about 17 kg.cm./mm.<sup>2</sup>. Lancashire iron of the composition mentioned above, without the nickel, has a maximum tensile strength of about 30 kg./mm.<sup>2</sup> and an elastic limit of about 17 kg./mm.<sup>2</sup>. Thus the nickel has effected a material increase in 75 the maximum tensile strength and also in the elastic limit of the product. And as for usual Lancashire iron the contraction seldom reaches more than 60-70% and the impact test 12-14 kg. cm./mm.<sup>2</sup>, the use of the 80 nickel has also effected a considerable increase in these quantities of the product.

In the problem in question as in many other respects cobalt has proved to have qualities, which are similar to those of the nickel. 85 Thence it is possible to carry out the present invention with cobalt entirely or partly substituted for the nickel.

For some purposes it may be convenient to alloy with the wrought iron besides the 90 nickel or the cobalt also a small quantity of copper. To the other good qualities the use of copper adds an increased resistance against rust.

I claim as my invention:

1. The process of manufacturing wrought iron consisting in heating nickeliferous pig

iron and puddling the same in a manner to produce a wrought iron to increase the usual tensile strength and elastic limit thereof without decreasing its welding and contraction capacities.

2. The process of manufacturing wrought iron consisting in adding a predetermined amount of nickel to ordinary pig iron and

then heating the mass and so puddling the same as to produce a wrought iron of increased tensile strength and elastic limit without decreasing its welding and contraction capacities.

In witness whereof, I have hereunto signed my name.

GEORG GUDE GEDDA.